

## 1

3,295,999

**PROCESS OF CHEMICAL METAL PLATING AND BATHS THEREFOR**

Heinz Günter Klein, Cologne-Deutz, and Eberhard Zirngiebl, Cologne-Flittard, Germany, assignors to Farbenfabriken Bayer Aktiengesellschaft, Leverkusen, Germany, a corporation of Germany  
 No Drawing. Filed Dec. 12, 1961, Ser. No. 158,873  
 Claims priority, application Germany, Dec. 31, 1960,  
 F 32,879

5 Claims. (Cl. 106—1)

The present invention relates to improved processes of chemical metal plating of metal or plastic articles employing bath with boron compounds with reducing agents and to improved baths therefor.

Chemical plating baths for the production of metal coatings on metal or plastic surfaces are known. As reducing agents there are used for this purpose sodium hypophosphite, alkali metal borohydride or boron compounds which carry 1 to 3 hydrogen atoms at the boron atom. The reduction with sodium hypophosphite is expediently carried out in the presence of buffer substances such as sodium citrate, sodium tartrate etc. When an alkali metal borohydride, such as sodium borohydride ( $\text{NaBH}_4$ ), is used as reducing agent, the process is carried out in aqueous alkaline solutions with the addition of complex formers such as ammonia, ethanolamine etc. Organic borohydride compounds with 1 to 3 H-atoms at the boron atom, for example

Borazanes (amine boranes), having the formula



Borazenes, having the formula  $\text{R}_2\text{N}=\text{BR}_2$

Borazines, having the formula  $\text{RN}=\text{BH}$

Borazoles, having the formula  $(\text{RN}-\text{BR})_3$

(wherein R represents alkyl, aryl or H, but at least one of the substituents at the B atom is H)

may be used in acidic as well as in aqueous alkaline or aqueous solutions. Here also buffer substances are used in acidic solutions, complex formers and possibly buffer substances in alkaline solutions.

Compared with the process using sodium hypophosphite, the chemical plating with alkali metal borohydride is substantially more economical, although in the hitherto known processes the reduction yield according to the equation



amounts only to about 20%.

The object of the invention is to provide baths for depositing metals on plastic or metal surfaces, which contain salts of the metals to be deposited and borohydride compounds with 1 to 4 hydrogen atoms directly linked with boron, and are characterized by a content of at least one element of Groups IIb, IIIb, IVb, Vb and/or VIb of the Periodic System of Elements. (See Lehrbuch für anorganische Chemie, edited by E. Wiberg, 37–39, edition 1956, page 443). Moreover, acidic baths contain buffer substances known as such, alkaline baths contain complex formers and, if desired, buffer substances.

The present invention is predicated upon the discovery that by the addition of compounds of elements of Groups IIb, IIIb, IVb, Vb and/or VIb of the Periodic System to plating baths containing as reducing agent borohydride compounds with 1 to 4 H-atoms at the boron atom, the reduction yields and/or plating rate are substantially increased. For example, additions of thallium nitrate to a chemical plating bath containing sodium borohydride as reducing agent, lead to reduction yields of 43% of the theoretical; an addition of stannous chloride to a bath

## 2

of the same composition gives reduction yields of 37% of the theoretical. With plating baths containing  $\text{N},\text{N}'$ -diethylborazane as reducing agent and giving a reduction yield of about 19% of the theoretical according to the equation:



an addition of, for example 300 mg. of  $\text{Ti}_2\text{HAsO}_4$  leads to reduction yields of 27%.

The plating rates are doubled or even tripled. For example, in an alkali metal borohydride bath without addition and with the use of 0.6 g.  $\text{NaBH}_4$  per litre and a ratio surface is  $\text{sq. cm.}/\text{bath volume in cc.} = 0.4$   $\text{NaBH}_4$  can no longer be detected only after 40 minutes of plating; with an addition of 200 mg. of  $\text{SnCl}_2 \cdot 2\text{H}_2\text{O}$ /litre to a bath of the same composition, the plating is already terminated after 15 minutes.

At certain concentrations, the metal additives are more over excellent lustre formers.

The elements of Groups IIb, IIIb, IVb, Vb and/or VIb of the Periodic System, such as nickel, cobalt, iron, zinc, arsenic, thallium, tin, cadmium or lead, can be added to the plating bath in the form of their dissolved salts, e.g. chlorides, sulphates, nitrates, acetates etc., individually or in combination with one another. It is immaterial whether the additive is added to the plating bath as cation, e.g.  $\text{SnCl}_2 \cdot 2\text{H}_2\text{O}$ ; as anion, e.g. sodium arsenate, or as salt of two effective elements, e.g.

30  $\text{TiHAsO}_4$ . A combination of two or more compounds as additive to plating baths is often advantageous. For example,  $\text{As}_2\text{O}_3$ , when added to a borohydride plating bath in an alkaline solution, yields reduction results of 30% of the theoretical only after an addition of 100 mg. 35  $\text{As}_2\text{O}_3$ /litre, whereas a combination with thallium added as  $\text{Ti}_2\text{HAsO}_4$  yields results of more than 40% of the theoretical already at 60 mg./litre. This effect of increased reduction yield and plating rate is surprising in so far as it is known from the literature that heavy metal salts decompose alkali metal borohydride solutions.

Metals, such as nickel, copper alloys, aluminum, iron as well as plastic material such as articles from acetyl cellulose, cellulose-acetobutyrate, polyvinylchloride, or polyethylene, can be plated with these new baths. The 45 content of the baths of salts of the plating metals such as sulphates, chlorides, acetates etc. of, for example, nickel, cobalt, iron, zinc etc., corresponds to the values already known for borohydride- or borazane-containing baths.

The plating metal salt concentration of the bath solution is about 30 g./litre and the boron compound concentration being about 0.1–10 g./litre to a ratio surface in  $\text{cm.}^2/\text{bath volume in cm.}^3 = 0.4$ . The absolute concentration of the boron compound in the bath expressed in mol/litre is within the range of 0.01–1.5, the molar ratio 55 of the metal salt of the plating metal to the boron compound in said bath is within the range 0.01–2.0 (metal salt/boron compound = 0.01–2.0) and the molar ratio of the metal salt of the plating metal to the salt or double-salt of elements of Group IIb, IIIb, IVb, Vb and VIb of the 60 Periodic System is within the range 0.001–0.1 (metal salt/ double salt = 0.001–0.1).

As reducing agents for the chemical depositing of metal there can be used for example:

(1) Alkali metal borohydrides such as sodium borohydride;

(2) Water-soluble B-H compounds, e.g.,  $\text{N},\text{N}',\text{N}''$ -trimethylborazane,  $\text{N},\text{N}'$ -dimethylborazane,  $\text{N},\text{N}'$ -dimethylborazene;

(3) B-H compounds which have been rendered water-soluble by the addition of solubilizers, e.g.,  $\text{N},\text{N}'$ -diethylborazane,  $\text{N}$ -isopropyl-borazene,  $\text{N}$ -isopropyl-borazine,  $\text{N}$ -

trimethylborazole. Solubilizers are, for example, methanol, dioxan, etc.

As buffer substances for these plating baths there may be used, for example, sodium acetate, sodium citrate, sodium tartrate etc.

Suitable complex formers are, for example, ammonia, ethylene diamine, ethanolamine etc.

The chemical plating of metal or plastic surfaces in the new plating baths presents advantages as follows:

(a) Improved utilisation of the reducing agent and thus reducing the costs of the process.

(b) Increased rate of depositing and thus reducing the time of stay of the object to be plated in the plating bath.

The coatings obtained on metal or plastic surfaces are smooth, brilliant and adherent.

The following examples are given for the purpose of illustrating the invention.

#### Example 1

1 litre of a plating bath consisting of 30 g./litre  $\text{NiCl}_2 \cdot 6\text{H}_2\text{O}$ , 40 g./litre  $\text{NaOH}$ , 50 g./litre  $\text{C}_2\text{H}_4(\text{NH}_2)_2$ , 70 mg./litre  $\text{TiNO}_3$  is heated to 90° C., 2 brass plates and 2 copper plates with a surface of 1 sq. dm./plate are suspended therein and 0.6 g.  $\text{NaBH}_4$ , dissolved in about 50 ml. of bath solution, are added. The  $\text{NaBH}_4$  content of the solution is established by iodometric analysis before the start and after termination of the plating. The plating is completed after about 20 minutes. A brilliant Ni-B coating of a total of 1.5187 g./4 sq. dm. is obtained on all plates, the consumption of  $\text{NaBH}_4$  being 0.5700 g. This corresponds to a  $\text{NaBH}_4$  reduction yield of 43.1%. With increasing addition of  $\text{TiNO}_3$  the following reduction yields are obtained:

| $\text{TiNO}_3$ /litre of bath liquor, mg.: | Reduction yield, percent |
|---------------------------------------------|--------------------------|
| 2                                           | 24.5                     |
| 20                                          | 36.0                     |
| 30                                          | 38.5                     |
| 40                                          | 41.0                     |
| 70                                          | 43.1                     |
| 120                                         | 43.2                     |
| 140                                         | 43.4                     |
| 150                                         | 43.6                     |
| 200                                         | 42.8                     |

#### Example 2

To 1 litre of a plating bath of the composition of 30 g./litre  $\text{NiCl}_2 \cdot 6\text{H}_2\text{O}$ , 40 g./litre  $\text{NaOH}$  and 50 g./litre  $\text{C}_2\text{H}_4(\text{NH}_2)_2$ , heated to 90° C., 220 mg.  $\text{SnCl}_2 \cdot 2\text{H}_2\text{O}$  are added, 4 iron plates with a surface of 1 sq. dm./plate are suspended therein and 0.6 g.  $\text{NaBH}_4$ , dissolved in 50 ml. of bath solution, are added. The plating is terminated after 15 minutes. A brilliant nickel coating of a total of 1.2959 g. is obtained on all plates, the  $\text{NaBH}_4$  consumption being 0.5700 g. This corresponds to a reduction yield of 36.8%.

With increasing addition of  $\text{SnCl}_2 \cdot 2\text{H}_2\text{O}$  the following reduction yields are obtained:

| $\text{SnCl}_2 \cdot 2\text{H}_2\text{O}$ /litre of bath liquor, mg.: | Reduction yield, percent |
|-----------------------------------------------------------------------|--------------------------|
| 2                                                                     | 21.0                     |
| 20                                                                    | 22.0                     |
| 40                                                                    | 22.5                     |
| 60                                                                    | 23.0                     |
| 110                                                                   | 24.4                     |
| 140                                                                   | 28.5                     |
| 160                                                                   | 30.3                     |
| 200                                                                   | 34.9                     |
| 220                                                                   | 36.8                     |
| 250                                                                   | 37.7                     |
| 300                                                                   | 38.8                     |
| 320                                                                   | 38.7                     |

#### Example 3

From a plating bath as described in Examples 2, the following reduction yields are obtained by the addition of increasing amounts of  $\text{As}_2\text{O}_3$  using a surface/volume ratio of 0.4:

| Mg. $\text{As}_2\text{O}_3$ /litre bath liquor: | Reducing agent, percent |
|-------------------------------------------------|-------------------------|
| 2                                               | 21.8                    |
| 10                                              | 23.8                    |
| 20                                              | 24.8                    |
| 45                                              | 25.5                    |
| 50                                              | 26.0                    |
| 60                                              | 26.1                    |
| 70                                              | 26.5                    |
| 85                                              | 27.8                    |
| 100                                             | 30.5                    |

#### Example 4

Acetyl cellulose foils are treated successively in the following baths:

(a) 100 g. of sodium hydroxide+0.3 g. of wetting agent+900 g. of water, time of stay: 5 minutes, temperature 50–60° C.

(b) 100 g./litre of stannous chloride+200 cc./litre of conc. hydrochloric acid+0.2 g. of wetting agent, time of stay: 5 minutes, temperature 50–60° C.

(c) 0.5 g./litre of palladium chloride+10 cc./litre of conc. hydrochloric acid, time of stay 5 minutes, temperature 20–30° C.

Four foils with a thickness of  $100\mu$  treated in this way are cut so that their surface amounts to 1 sq. dm./foil and suspended in a plating bath of the composition given in Example 2. 180 mg. of  $\text{SbCl}_3$  are added to the plating bath which is heated to 90° C. and 0.6 g.  $\text{NaBH}_4$ , dissolved in 50 ml. of bath solution, are added. The surface in sq.cm./bath volume in cc. ratio is 0.4. A brilliant adherent nickel-boron coating of a total of 1.3114 g. is obtained on all foils, the  $\text{NaBH}_4$  consumption being 0.5890 g. This corresponds to a reduction yield of 35.9%.

With increasing  $\text{SbCl}_3$  content in the plating bath the following reduction yields are obtained. The surface/volume ratio is 0.4.

| Mg. $\text{SbCl}_3$ /litre bath liquor: | Reduction yield, percent |
|-----------------------------------------|--------------------------|
| 2                                       | 19.6                     |
| 20                                      | 21.7                     |
| 50                                      | 25.2                     |
| 70                                      | 27.1                     |
| 100                                     | 30.0                     |
| 130                                     | 32.6                     |
| 150                                     | 33.8                     |
| 180                                     | 35.9                     |
| 200                                     | 36.5                     |
| 240                                     | 38.0                     |

#### Example 5

By the addition of  $\text{PbCl}_2$ ,  $\text{SeO}_2$ ,  $\text{TeO}_2$ ,  $\text{CdCl}_2$  to 1 litre each of plating bath as indicated in Example 2, the following reduction yields are obtained using a surface/volume ratio of 0.4:

| (a) Mg. $\text{PbCl}_2$ /1 litre of bath liquor: | Percent reduction yield |
|--------------------------------------------------|-------------------------|
| 4.0                                              | 22.8                    |
| 6.0                                              | 30.0                    |
| 10.0                                             | 35.2                    |
| 20.0                                             | 32.6                    |
| 60.0                                             | 32.4                    |
| 100.0                                            | 32.2                    |

| (b) Mg. $\text{SeO}_2$ /1 litre of bath liquor: | Percent reduction yield |
|-------------------------------------------------|-------------------------|
| 0.4                                             | 21.4                    |
| 0.8                                             | 23.6                    |
| 1.0                                             | 24.6                    |
| 2.0                                             | 26.2                    |
| 4.0                                             | 25.4                    |
| 6.0                                             | 22.0                    |

| (c) Mg. $\text{TeO}_2$ /1 litre of bath liquor: | Percent reduction yield |
|-------------------------------------------------|-------------------------|
| 2.0                                             | 22.8                    |
| 4.0                                             | 24.8                    |
| 6.0                                             | 27.0                    |
| 8.0                                             | 30.0                    |
| 10.0                                            | 29.6                    |

| (d) Mg. $\text{CdCl}_2$ /1 litre of bath liquor: | Percent reduction yield |
|--------------------------------------------------|-------------------------|
| 2.0                                              | 22.0                    |
| 100.0                                            | 27.5                    |
| 200.0                                            | 29.0                    |
| 250.0                                            | 29.2                    |
| 350.0                                            | 28.8                    |

*Example 6*

By the addition of  $\text{TINO}_3$  and  $\text{SnCl}_2 \cdot 2\text{H}_2\text{O}$  in a proportion by weight of 1:1 to 1 litre of a plating bath as described in Example 2 using a surface/volume ratio = 0.4 there are obtained the following reduction yields:

| Mg. $(\text{SnCl}_2 \cdot 2\text{H}_2\text{O} \text{ TINO}_3)$ (1:1) per litre of bath liquor: | Percent reduction yield |
|------------------------------------------------------------------------------------------------|-------------------------|
| 2                                                                                              | 22.8                    |
| 20                                                                                             | 30.0                    |
| 50                                                                                             | 38.4                    |
| 80                                                                                             | 42.1                    |
| 100                                                                                            | 43.0                    |
| 150                                                                                            | 43.5                    |
| 200                                                                                            | 43.0                    |
| 250                                                                                            | 43.3                    |

*Example 7*

An addition of  $\text{Ti}_2\text{HAsO}_4$  to 1 litre of a plating bath as described in Example 2 using a surface/volume ratio = 0.4 gives the following reduction yields:

| Mg. $\text{Ti}_2\text{HAsO}_4$ per litre of bath liquor: | Percent reduction yield |
|----------------------------------------------------------|-------------------------|
| 2                                                        | 23.3                    |
| 20                                                       | 32.6                    |
| 50                                                       | 37.9                    |
| 60                                                       | 40.7                    |
| 80                                                       | 41.0                    |
| 100                                                      | 42.2                    |
| 120                                                      | 41.5                    |
| 150                                                      | 43.4                    |

*Example 8*

To a plating bath of the composition of 30 g.  $\text{NiCl}_2 \cdot 6\text{H}_2\text{O}$ , 5 g. of ammonium chloride, 10 g. of sodium citrate, 20 g. of sodium acetate and 950 cc. of water, heated to 70° C., are added 250 mg. of thallium nitrate and 4 metal plates with a surface of 1 sq. dm./plate are suspended therein. The pH value is 5.0. After the addition of 50 ml. of a solution of 3.400 g. of N,N'-diethylborazane in methanol, a highly brilliant coating of a total of 1.9052 g. Ni is obtained on all plates within 30 minutes. This corresponds to a reduction yield of 27.8% of the theoretical.

With increasing  $\text{TINO}_3$  addition, the following reduction yields are obtained (surface/volume=0.4):

| Mg. $\text{TINO}_3$ : | Percent reduction yield |
|-----------------------|-------------------------|
| 5                     | 19.25                   |
| 10                    | 19.55                   |
| 20                    | 20.00                   |
| 50                    | 20.60                   |
| 80                    | 22.10                   |
| 100                   | 23.50                   |
| 150                   | 24.00                   |
| 200                   | 25.90                   |
| 250                   | 27.30                   |
| 300                   | 27.80                   |
|                       | 28.20                   |

*Example 9*

Four foils of cellulose-acetobutyrate with a surface of 1 sq. dm./foil and a thickness of 100 $\mu$ , pre-treated as described in Example 4, are suspended in a plating bath of the composition 30 g.  $\text{NiCl}_2 \cdot 6\text{H}_2\text{O}$ , 5 g. of ammonium chloride, 10 g. of sodium citrate, 20 g. of sodium acetate and 950 cc. of water at 70° C.

200 mg. of  $\text{Ti}_2\text{HAsO}_4$  and 50 ml. of a solution of 3.1920 g. of N,N'-diethylborazane in methanol are added thereto. The pH value is 5. A highly brilliant Ni-coating of a total of 1.6883 g. is obtained on all four foils. This corresponds to a reduction yield of 26.2% of the theoretical.

With increasing  $\text{Ti}_2\text{HAsO}_4$  addition, the following reduction yields are obtained:

| Mg. $\text{Ti}_2\text{HAsO}_4$ per litre of bath liquor: | Percent reduction yield |
|----------------------------------------------------------|-------------------------|
| —                                                        | 19.2                    |
| 20                                                       | 21.5                    |
| 50                                                       | 22.7                    |
| 80                                                       | 24.3                    |
| 120                                                      | 25.2                    |
| 150                                                      | 25.8                    |
| 200                                                      | 26.2                    |
| 350                                                      | 27.6                    |
| 750                                                      | 31.7                    |
| 900                                                      | 34.5                    |

*Example 10*

By the addition of (a)  $\text{SnCl}_2 \cdot 2\text{H}_2\text{O}$  (b) arsenous acid to a plating bath as described in Example 8, the following reduction yields are obtained using a surface/volume ratio = 0.4:

| (a) Mg. $\text{SnCl}_2 \cdot 2\text{H}_2\text{O}$ /1 litre of bath liquor: | Percent reduction yield |
|----------------------------------------------------------------------------|-------------------------|
| 20                                                                         | 20.5                    |
| 50                                                                         | 21.4                    |
| 100                                                                        | 22.7                    |
| 200                                                                        | 25.0                    |
| 400                                                                        | 28.4                    |
| 750                                                                        | 33.6                    |

  

| (b) Mg. arsenous acid litre of bath liquor: | Percent reduction yield |
|---------------------------------------------|-------------------------|
| 20                                          | 20.0                    |
| 50                                          | 20.4                    |
| 100                                         | 21.8                    |
| 150                                         | 25.0                    |
| 200                                         | 29.1                    |
| 250                                         | 34.3                    |

We claim:

1. An aqueous metal and plastic plating bath for plating by chemical reduction consisting essentially of 30 g./l.  $\text{NiCl}_2 \cdot 6\text{H}_2\text{O}$ , 50 g./l.  $\text{C}_2\text{H}_4(\text{NH}_2)_2$ , 2-200 mg./l.  $\text{TINO}_3$  and 0.6 g./l.  $\text{NaBH}_4$ .
2. An aqueous metal and plastic plating bath for plating by chemical reduction, consisting of 30 g./l.  $\text{NiCl}_2 \cdot 6\text{H}_2\text{O}$ , 50 g./l.  $\text{C}_2\text{H}_4(\text{NH}_2)_2$ , 20-250 mg./l. of a mixture of  $\text{TINO}_3$  and  $\text{SnCl}_2 \cdot 2\text{H}_2\text{O}$  in a proportion by weight of 1:1, and 0.6 g./l.  $\text{NaBH}_4$ .
3. An aqueous metal and plastic plating bath for plating by chemical reduction, consisting of 30 g./l.  $\text{NiCl}_2 \cdot 6\text{H}_2\text{O}$ , 50 g./l.  $\text{C}_2\text{H}_4(\text{NH}_2)_2$ , 20-150 mg./l.  $\text{Ti}_2\text{HAsO}_4$ , and 0.6 g./l.  $\text{NaBH}_4$ .
4. An aqueous metal and plastic plating bath for plating by chemical reduction consisting essentially of 30 g.  $\text{NiCl}_2 \cdot 6\text{H}_2\text{O}$ , 5 g. ammonium chloride, 10 g. sodium citrate, 20 g. sodium acetate, 250 mg. thallium nitrate, 3.4 g. N,N'-diethylborazane in the form of its solution in 50 ml. methanol and 950 cc. of water.

5. An aqueous metal and plastic plating bath for plating by chemical reduction consisting essentially of 30 g.  $\text{NiCl}_2 \cdot 6\text{H}_2\text{O}$ , 5 g. ammonium chloride, 10 g. sodium citrate, 20 g. sodium acetate, 20-900 mg.  $\text{Ti}_2\text{HAsO}_4$ , 3.1920 g. N,N'-diethylborazane in the form of its solution in 5 methanol, and 950 cc. of water.

**References Cited by the Examiner**

**UNITED STATES PATENTS**

|           |         |                    |           |
|-----------|---------|--------------------|-----------|
| 2,844,530 | 7/1958  | Wesley et al.      | 204-49    |
| 2,884,344 | 4/1959  | Ramirez            | 106-1 X   |
| 2,898,379 | 7/1959  | Chamberlain et al. | 260-583 X |
| 2,990,296 | 6/1961  | Hoke               | 106-1 X   |
| 2,994,369 | 8/1961  | Carlen             | 106-1     |
| 3,062,666 | 11/1962 | McLeod             | 106-1     |
| 3,096,182 | 7/1963  | Berzins            | 106-1     |

10

15

Lange's Handbook of Chemistry, pages 56 and 57, 9th edition, 1956.

Wm. Scheckter, C. B. Jackson, and Roy M. Adams: "Boron Hydrides and Related Compounds," 2nd ed., Cal-  
lery Chemical Company, 1954.

**MORRIS LIEBLMAN, Primary Examiner.**

**JOSEPH REBOLD, ALEXANDER H. BRODMERKEL,**  
**Examiners.**

**J. E. CARSON, J. E. CALLAGHAN, L. B. HAYES,**  
**Assistant Examiners.**

**FOREIGN PATENTS**

626,999 9/1961 Canada.  
836,480 6/1960 Great Britain.

**OTHER REFERENCES**